

# UNITED STATES PATENT OFFICE.

SAMUEL T. G. SMITH, OF ST. LOUIS, MISSOURI.

## METHOD OF MAKING SMOOTH CASTINGS.

No Drawing.

Application filed May 24, 1926. Serial No. 111,374.

This invention relates to a method of making smooth castings.

In making castings by the use of molds wherein the mold walls comprise sand or other finely divided mineral particles, the molten metal has a tendency to penetrate the walls of the molds, with the result that the surface of the casting is rough. After the casting is removed from the mold it is necessary to smooth the casting by machining or other treatment resulting in increased cost of production.

The present invention provides a method whereby penetration of the mold walls by the molten metal may be prevented so that castings may be formed with comparatively smooth surfaces, with the result that the operations are facilitated and the amount of time and cost required to obtain the desired smoothness are largely reduced.

I obtain these desirable and beneficial results by facing the walls of the molds or other casting agencies, such as cores, with powdered barytes ( $BaSO_4$ ). The walls of the casting agencies so treated resist the tendency of the molten metals to penetrate the walls and a much smoother casting is obtained than can be produced by the usual casting agencies having walls formed of sand or other mineral particles.

What I claim and desire to secure by Letters Patent is:—

1. A facing composed of powdered barytes ( $BaSO_4$ ) for the walls of molds and cores used as casting agencies.

2. A facing for the walls of molds and cores used as casting agencies, composed of barytes ( $BaSO_4$ ) adhering to the walls of said casting agencies.

SAMUEL T. G. SMITH.